

July 11, 1939.

E. S. CORNELL, JR.

2,165,454

METHOD OF PRODUCING BRANCH FITTINGS

Filed July 27, 1937

2 Sheets-Sheet 1



INVENTOR

Edward S. Cornell, Jr.

*Henry J. Luce*  
HIS ATTORNEY

July 11, 1939.

E. S. CORNELL, JR.

2,165,454

METHOD OF PRODUCING BRANCH FITTINGS

Filed July 27, 1937

2 Sheets-Sheet 2

Fig. 6.



Fig. 7.



Fig. 8.



INVENTOR  
Edward S. Cornell, Jr.  
*Henry J. Luske*  
HIS ATTORNEY

Patented July 11, 1939

2,165,454

# UNITED STATES PATENT OFFICE

2,165,454

## METHOD OF PRODUCING BRANCH FITTINGS

Edward S. Cornell, Jr., Larchmont, N. Y., assignor, by mesne assignments, to American Radiator & Standard Sanitary Corporation, New York, N. Y., a corporation of Delaware

Application July 27, 1937, Serial No. 155,884

4 Claims. (Cl. 29—157)

My present invention relates to the production of T and kindred fittings from preformed sections.

More particularly, my present invention is directed to T and kindred fittings formed of metal 5 of predominant copper content, a characteristic of my method residing in the treatment of the preformed section pursuant to appropriate procedure by cold working, that is to say, in the absence of supplied heat, thereby obviating the 10 chemical formation of cuprous oxide and/or other deleterious.

Specifically, pursuant to the more preferred procedure of my invention for the production of a T, a rod of the desired copper content is preformed by extrusion to be preshaped in respect 15 to general configuration, advantageously of a general T-configuration, and possessing dimensional characteristics, whereby after severing a section from such rod to have a cubical content 20 corresponding to the cubical content of the eventual T or other fitting, such section is subjected to successive stages of cold working, as in an appropriate die and appropriate sets of punches and plugs, or equivalent; resulting eventually in the desired fitting of desired configurations and 25 dimensions of its component parts, the eventual fitting and its component parts being eventually and at all stages of treatment wholly integral.

As appears from the hereinafter appearing particulars, the section, say of T-configuration 30 for the formation of a T, is of polyhedral configuration, preferably symmetrical, the dimensions of length, height and thickness being substantially less than the ultimate dimensions of the eventual T, the dimensions of the diagonals of the T-configurated section, however, corresponding substantially to the outer diameter of the central body portion of the eventual T. Accordingly, when the stated T-configurated section 35 is placed in a suitably apertured female die, the aperture diameter of which is substantially the outer diameter of the T body, the stated dimensional characteristics of the T-configurated section afford accurate placement of the same within 40 the apertures of the die, and retain the section in proper position relative to the male die members prior to and during the stage of cold working.

Further features and objects of my invention 45 will be more fully understood from the following detail description and accompanying drawings, in which

Fig. 1 is a vertical sectional view of a typical product produced pursuant to my invention.

Fig. 2 is an "exploded" view in perspective, 50 showing an indefinite length of predetermined stock, and a severed section thereof, the length of stock bearing indications of lines of successive severing, utilized in carrying out a preferred 55 form of my invention.

Fig. 3 is an elevation in vertical section through an appropriate die, illustrating in superposition the eventual T fitting, compared with Fig. 1, and a severed section similar to Fig. 2, from which the T fitting is to be produced.

Fig. 4 is an end view of Fig. 3.

Fig. 5 is a vertical central section, illustrating an intermediate stage of operation employing appropriate punches and/or stops, pursuant to my method.

Figs. 6, 7 and 8 are respectively successive stages of operation subsequent to the stage of Fig. 5.

Referring to the drawings, I have indicated in Fig. 1 at 10 a preferred type of wholly integral wrought copper T fitting, such as is described and claimed, per se, in my U. S. Patent No. 2,025,973, December 31, 1935, entitled Hollow metal bodies and methods of making same.

Assuming the wrought copper T fitting to be 20 of the type illustrated in Fig. 1, pursuant to my present method, I provide a preshaped indefinite length of rod 11, formed preferably by extrusion, and preferably, also, of commercially pure copper or of alloy of predominantly high copper content. Such rod 11 comprises in essentials: a general T configuration (shown inverted for convenience); a mean height of base of the T-rod indicated by the double arrowed line 12 less than the outer diameter indicated in Fig. 1 by the double arrowed line 13 of each body end opening 14 of the T fitting 10; a mean width of base of the T-rod 11, indicated by the double arrowed line 15, Fig. 2, less than the over-all length of the body of the T fitting 10, indicated by the double arrowed line 16, see Fig. 1; a mean height of the T-rod 11 less than the height indicated by the double arrowed line 18 of the lateral opening 19 of the T fitting 10, see Fig. 1, and a mean width indicated by the double arrowed line 20 of the stem of the T-rod 11, see Fig. 2, less than the outer diameter indicated by the double arrowed line 21 of the lateral opening 19 of the T fitting 10, see Fig. 1. Preferably, such T-rod 11 is pre-shaped, preferably simultaneously with its general T formation by extrusion, with an arcuate groove indicated at 22, see Fig. 2.

Such general T-shaped rod 11 may be severed into sections. Lines of severing of such sections are predetermined from the factor of the cubical content of each section in correspondence to the cubical content of the eventual T fitting, assuming the above noted dimensional factors. The separate section 11' appearing in Fig. 2, indicates the procedure of severing, which procedure may be further carried out by severing at the indicated dot and dash lines 11a, 11a, etc., for producing duplicate T fittings. If preferred, the stated sections 11' and duplicates thereof may be preformed separately.

A direct comparison of relative exterior and interior dimensions and exterior and interior configurations of the section 11' with the eventual T fitting produced pursuant to my invention, 5 appears from the showing of Fig. 3.

A preferred procedure, in carrying out my method, of producing individual T fittings from T formed sections, such as the section 11', is indicated in Figs. 4, 5, 6, 7 and 8, which depict 10 successive advantageously related stages.

The fitting shown in Fig. 1 is illustrative of a "sweat jointed" T, contemplating the use of soldered, rather than pipe threaded, joints in its ultimate installation in a piping system.

Accordingly, the inner surfaces of the socket 15 ends 14, 19 are preferably smooth and of uniform diameter throughout, it being intended that their inner diameters be so related to the outer diameter of the pipe or fitting forming the male member of the joint that provision is made for clearance therebetween, accommodating capillary and/or surface flow of the bonding medium while in the status of fluidity. Preferably, shoulders 14a, 19a delineate between the respective socket 20 ends and the body 10c of the T, said shoulders 25 incidentally serving as stops by which to gauge the insertion of the pipes.

It will be understood that this invention is 30 equally applicable to the production of fittings intended for pipe-threaded connection; it being necessary only to provide additional wall thickness at the sockets to accommodate thread cutting.

The invention contemplates the formation of 35 the fitting by cold-working processes which eliminate, as far as is practicable, the use of drilling or milling operations, thus minimizing wastage of material. In accordance with this invention, therefore, an interiorly hollow product is fabricated by cold-flow displacement of a solid mass 40 of metal, usefully employing substantially all of the metal in the said mass in attaining the ultimate objective; and minimizing operations addressed purely to "finishing" the fitting by causing 45 the metal, by such cold flow, to conform to the configuration of cooperating male and female dies.

Advantageously, the fitting is formed from the mass 11' by subjecting the said mass to punch 50 and die operations inducing compressive stresses in the said mass exceeding the pressure of fluidity of the material of the mass, whereupon, cold plastic movement of the said material occurs.

Figures 3 and 4 show a two-part female die 55 23, having a cavity 10a which defines the outer configuration of the finished fitting 10; access to the cavity being the cylindrical channels 24. The mass 11' is placed within the cavity 10a, as illustrated. As previously stated the overall 60 dimensions of the said mass are appreciably less than the ultimate dimensions of the fitting, except that the diagonal of the end section of the mass 11', see Figure 4, may be equal to the outside diameter of the central body portion 10c of the completed T. By so dimensioning the mass 11', its centralized location within the die 23 may be conveniently established.

As appears from Figs. 3, 4 and 5, by provision 70 of the diagonal dimension of the section 11' corresponding substantially to the diameter of the die aperture, the mass 11' is accurately positioned within the die apertures, preparatory for engagement therewith by the male dies 25, 25, 26.

It is understood that the two halves of the 75 die 23 are suitably clamped together, the pins

23a cooperating with suitable recesses (not shown) to maintain the transverse alignment of the die, in accordance with established practice.

Cold flow of the metal of the mass 11' is accomplished in coordinated steps, of which the first advantageously comprises simultaneously applying pressure, by means of a powerful quick-acting press, to the outer ends of the punches or male dies 25, which act to form the run of the T 10, and 26, which operates on the lateral 10 thereof. The said dies have shanks 25a, 26a which closely, but slidably, fit the aforementioned channels 24 of the die 23. Advantageously, the dies 25, 26 have bluntly rounded ends, to induce the cold flow of the metal with minimum friction between the flowing metal and the dies. The shape of the tip of the die 26 may conform to the arcuate groove 22, thereby serving to maintain the centralized position of the mass 11' of the cavity 10a during the first stages of the pressure application. It is to be noted from Figure 5 that the said dies include a shoulder 25b, 26b, the diameter of which may be equivalent to the interior diameter of the body portion 10c of the fitting 10.

The pressure exerted by the inwardly driving dies 25, 26 causes the integral metal of the mass 11' to flow or move outwardly within the limits of the diameter of the cavity 10a, and rearwardly with respect to the said dies. Cold plastic deformation of the metal of the mass 11', and particularly the central portion or core thereof, alone brings the said mass into an approximation of the desired final form.

Figure 6 illustrates the substitution for the 35 male dies 25, 26 of a second set of dies 27, 28 arranged to complete the plastic flow, and to form the essentially smooth inner-wall surfaces of the fitting. The heads 27a of the dies 27 are preferably cylindrical, with an outside diameter equivalent to the diameter of the aforementioned central portion 10c of the run of the completed fitting 10. The smoothly cylindrical dyeshanks 27b suitably form smooth-walled interiors of the ends 14. The shoulder 27c of each die 27 40 is arranged to cooperate with the cavity 10a of the die 23 in forming the gauging shoulders 14a of the fitting 10. The shank 28b of vertical die 28 is equal in diameter to the socket 19 of the fitting 10, and its rounded end guides the 45 upward flow of the metal into the walls of the said socket.

By application of suitable cold-flow-inducing pressures to the dies 27, 28, the cold flow of the metal of the mass 11' is completed, as indicated 55 in Figure 6, which illustrates the complete conformation of the metal to the confines of the die cavity. As indicated in Figure 6, substantially all of the metal of the mass 11' has been usefully employed, surplus material of the mass 11' appearing merely as a thin-walled dam or membrane 31, and a thin partition 32 at the base of the lateral 19. The outer configuration of the entire fitting 10 is complete, except for clipping or otherwise removing the fins which 60 may result from the penetration of the metal of the mass 11' between the halves of the die 23.

As appears from the above, the pre-shaped work is a solid mass having an exterior configuration conforming generally to the desired 70 exterior configuration of the desired fitting, the desired fitting being attained by applying pressure, preferably by suitable opposingly related die members within a suitable female die, where-by the metal of such mass is caused to flow out- 75

wardly, the walls of the female die member serving to guide the flow of the metal to attain the desired exterior configuration and the desired exterior dimensions, the lateral die members serving to control the flow of the metal interiorly of the mass to attain the desired interior configuration and the desired interior dimensions of the fitting.

Figure 7 illustrates a step in the completion 10 of the process, wherein the mass 11', now transformed solely by cold plastic metal flow into a representation of the ultimate product 10, and still remaining within the confines of the die 23, is subjected to a brief drilling operation to remove 15 the membrane 31. Reaming or smoothing the horizontal central portion 10c of the fitting or of the terminals 14 thereof is rendered unnecessary, as the metal of the mass 11' has conformed both to the configuration of the cavity 10a, and to the 20 smooth surfaces of the dies 21.

The penetration of the partition 32 may include the application of a combined drill and reamer 33, which at once drills through the said partition and completes the formation of the cylindrical, smooth walled interior surface of the 25 socket 19, and provides the gauging shoulder 19a thereof.

Whereas I have described my invention by reference to specific forms thereof, it will be 30 understood that many changes and modifications may be made without departing from the spirit of the invention.

I claim:

1. The method of producing a lateral branch 35 hollow fitting of cold-wrought metal of predominant copper content, the fitting having predetermined exterior and interior configurations and dimensions thereof, which comprises providing a polyhedral mass of such metal having an exterior configuration corresponding generally to the desired configuration of the desired fitting but having exterior dimensions less than the exterior dimensions of the desired fitting, a diagonal dimension of such polyhedral mass corresponding substantially to the diametrical dimension of the fitting desired to be produced, positioning such polyhedral mass in a suitable female die having an aperture of a diameter corresponding substantially to the stated diagonal dimension of such polyhedral mass, subjecting such polyhedral mass in cold state to pressure to cause flow of the metal in outward directions and giving rise to hollow interior formation within the mass and guiding the flow of the metal exteriorly to form the desired exterior configuration of the desired outer dimensions while controlling the flow of the metal to form the desired interior configuration of the desired interior dimensions.

2. The method of producing a lateral branch 60 hollow fitting of cold-wrought metal of predominant copper content, the fitting having predetermined exterior and interior configurations and dimensions thereof, which comprises providing a symmetrical polyhedral mass of such metal having a cubical content substantially equal to the cubical content of the metal of the desired fitting and further having an exterior configuration corresponding generally to the desired configuration of the desired fitting but having exterior dimensions less than the exterior dimensions of the desired fitting, a diagonal dimension of such symmetrical polyhedral mass corresponding substantially to the diametrical dimension of the fitting desired to be produced, positioning such symmetrical polyhedral mass in a suitable female die having an aperture of a diameter corresponding substantially to the stated diagonal dimension of such symmetrical polyhedral mass, subjecting such symmetrical polyhedral mass in cold state to pressure by opposingly related die members to cause flow of the metal in outward directions and giving rise to hollow interior formation within the mass and guiding the flow of the metal exteriorly to form the desired exterior configuration of the desired outer dimensions while controlling the flow of the metal to form the desired interior configuration of the desired interior dimensions.

dimension of the fitting desired to be produced, positioning such symmetrical polyhedral mass in a suitable female die having an aperture of a diameter corresponding substantially to the stated diagonal dimension of such symmetrical polyhedral mass, subjecting such symmetrical polyhedral mass in cold state to pressure to cause flow of the metal in outward directions and giving rise to hollow interior formation within the mass and guiding the flow of the metal exteriorly 10 to form the desired exterior configuration of the desired outer dimensions while controlling the flow of the metal to form the desired interior configuration of the desired interior dimensions.

3. The method of producing a lateral branch 15 hollow fitting of cold-wrought metal of predominant copper content, the fitting having predetermined exterior and interior configurations and dimensions thereof, which comprises providing a symmetrical polyhedral mass of such metal 20 having an exterior configuration corresponding generally to the desired configuration of the desired fitting but having exterior dimensions less than the exterior dimensions of the desired fitting, a diagonal dimension of such symmetrical polyhedral mass corresponding substantially to the diametrical dimension of the fitting desired to be produced, positioning such symmetrical polyhedral mass in a suitable female die having an aperture of a diameter corresponding substantially to the stated diagonal dimension of such symmetrical polyhedral mass, subjecting such symmetrical polyhedral mass in cold state to pressure by opposingly related die members to cause flow of the metal in outward directions and 25 giving rise to hollow interior formation within the mass and guiding the flow of the metal exteriorly to form the desired exterior configuration of the desired outer dimensions while controlling the flow of the metal to form the desired interior configuration of the desired interior dimensions.

4. The method of producing a lateral branch 30 hollow fitting of cold-wrought metal of predominant copper content, the fitting having predetermined exterior and interior configurations and dimensions thereof, which comprises providing a symmetrical polyhedral mass of such metal having a cubical content substantially equal to the cubical content of the metal of the desired fitting and further having an exterior configuration corresponding generally to the desired configuration of the desired fitting but having exterior dimensions less than the exterior dimensions of the desired fitting, a diagonal dimension of such symmetrical polyhedral mass corresponding substantially to the diametrical dimension of the fitting desired to be produced, positioning such symmetrical polyhedral mass in a suitable female die having an aperture of a diameter corresponding substantially to the stated diagonal dimension of such symmetrical polyhedral mass, subjecting such symmetrical polyhedral mass in cold state to pressure by opposingly related die members to cause flow of the metal in outward directions and giving rise to hollow interior formation within the mass and guiding the flow of the metal exteriorly to form the desired exterior configuration of the desired outer dimensions while controlling the flow of the metal to form the desired interior configuration of the desired interior dimensions.